

Patented July 3, 1928.

1,675,708

# UNITED STATES PATENT OFFICE.

NOAK VICTOR HYBINETTE, OF WILMINGTON, DELAWARE.

## ALLOY.

No Drawing. Application filed September 23, 1922, Serial No. 589,996. Renewed November 17, 1927.

This invention relates to improved alloys containing a preponderating amount of aluminum, together with small amounts of nickel and other metals, and with the nickel 5 in preponderating amount as compared with the other metals.

In my prior application Serial No. 587,583, filed September 11, 1922, I have described alloys of aluminum and nickel which 10 possess important advantages as compared with aluminum itself. According to the present invention, I make the alloys with the addition of other metals to the aluminum and nickel, these other metals being introduced in small quantity less than the amount 15 of the nickel. Among such other metals are iron, chromium, tungsten and molybdenum. When these other metals are present, the presence of copper is undesirable, and would 20 make the alloy red short or short even below 700° F. The presence of copper would also make the alloy poisonous and therefore unfit for use for cooking utensils. In making the new alloys, therefore, I add other metals to 25 the aluminum and nickel without adding copper.

The new alloys can be produced in the manner described in my said prior application, by adding the alloying metals to the 30 molten aluminum. My preferred composition of the alloy is as follows: Nickel from about 3 to about 6%; iron from about 0.5% to about 2%; and chromium, tungsten and molybdenum, either separately or together, 35 amounting to about 0.2% to about 1%; and with the remainder aluminum. Small amounts of other metals or elements may also be present which do not interfere with the desired valuable properties of the alloys; 40 for example, manganese, magnesium, silicon, etc. may be present in small amount. The presence of copper should be avoided since it is detrimental in the alloys of aluminum with metals of the iron group but a small 45 amount of copper may be substantially harmless.

The new alloys accordingly are made up of a preponderating amount of aluminum, while the nickel is also in preponderating 50 amount as compared with the other metals. These other metals include metals of the iron and chromium groups, and copper being excluded from the alloy. I believe that I am the first to discover the detrimental effect of copper in alloys of aluminum with metals of the iron group.

The new alloys, as compared with metallic aluminum, have a greatly increased tensile strength and elastic limit, as well as a greatly increased elongation. The new 60 alloys are capable of being rolled and worked into sheets and other shapes. The new alloys and articles made therefrom have a characteristic lustre and color different from that of any known aluminum alloy, 65 being more like nickel than aluminum in appearance.

Sheets of the new alloy can be used in making cooking utensils and other articles. The sheets are harder than aluminum but 70 nevertheless ductile while the drawing or working operation by which the sheets are produced and to which they are subjected tends to eliminate imperfections in the surface of the sheets instead of magnifying 75 them. The sheets of the alloy are sufficiently ductile to permit the forming of articles by various shapes by drawing, stamping and other mechanical processes of working. The new alloy can be used for 80 purposes where metallic aluminum is unsuitable or objectionable because of its softness and for purposes where nickel plated brass is now used. For example, the new alloy can be used for making automobile 85 parts such as the handles of doors, the caps of the hubs of wheels, etc.

### I claim:

1. An alloy of aluminum with metals of the iron group in which the aluminum forms 90 upwards of about 90% of the alloy, said alloy containing nickel and iron in small but substantial amount, and said alloy containing at least one of the following metals, namely, chromium, tungsten and molybdenum, in substantial amount less than 1%, said alloy being practically free from copper.

2. An alloy containing a preponderating amount of aluminum, from about 3 to about 100 6% of nickel, and from about 0.5% to about 2% of iron, said alloy being practically free from copper.

3. An alloy containing a preponderating amount of aluminum, from about 3 to about 105 6% of nickel, from about 0.5 to 2% of iron, and from 0.2 to 1% of at least one of the following metals, namely, chromium, tungsten and molybdenum.

In testimony whereof I affix my signature.

NOAK VICTOR HYBINETTE.